

March 21, 1939.

R. R. LAING

2,151,049

DRYING ROLL

Filed July 1, 1937



WITNESSES:

*Joseph A. Gangi*  
*Frank J. Murphy*

BY

INVENTOR  
RICHARD R. LAING.

*S. Edward Low*  
ATTORNEY.

## UNITED STATES PATENT OFFICE

2,151,049

## DRYING ROLL

Richard R. Laing, Fairfield, Conn., assignor to  
Aluminum Company of America, Pittsburgh,  
Pa., a corporation of Pennsylvania

Application July 1, 1937, Serial No. 151,441

7 Claims. (Cl. 34—24)

This invention relates to the manufacture of cellulose material, and more particularly to a method of drying cellulose material and to drying machinery used in its manufacture.

In the course of the manufacture of sheets or films of non-fibrous cellulose material, such as that sold under the name "Cellophane", it is customary to subject the sheets to a drying and stretching operation. This is ordinarily done by passing them over a succession of heated rolls having a somewhat tacky surface or a surface to which the sheets will adhere. The rolls are in the form of metal cylinders mounted to rotate about their longitudinal axes, and may be heated by any of a number of methods, although the method generally used is to run hot water through them.

Prior to my invention, iron and steel drying rolls having a coating of varnish have been used for this purpose. However, such rolls have presented several difficulties. The coating of varnish wears away in use and must be renewed comparatively frequently. Also, the adhesiveness of the varnish coating varies with the temperature of the roll; the colder the roll is, the less adhesive is its surface, so that it is difficult to obtain uniform results. Furthermore, the individual rolls do not heat uniformly throughout, the result being that the drying effect of any one roll on the cellulose material may vary, depending on what portion of the roll comes in contact with the material and on the temperature of that portion.

It has been proposed to make the rolls of aluminum because this metal conducts heat more readily and uniformly than iron or steel. However, such rolls have not been entirely satisfactory, chiefly because of the fact that in the course of its passage through the drying machinery, cellulose material sometimes becomes tangled among the rolls and must be cut away with sharp knives which frequently score the aluminum and raise burrs on the roll surfaces. These burrs mar the cellulose sheets which subsequently pass over them. Another difficulty encountered with aluminum rolls is that their external surface is corroded by the treating solutions present on the cellulose material, and their internal surface may be corroded by the water which heats the rolls, if this method of heating is used.

It is an object of my invention to provide an aluminum drying roll for use in the drying of cellulose films or sheets, the roll having an external surface which is of a type which will not be susceptible to burring by knife edges when cellu-

lose material must be cut away from the roll. Another object of the invention is to provide an aluminum drying roll having a hard, adherent, abrasion-resistant coating consisting substantially of aluminum oxide. A further object of my invention is to provide a method of drying cellulose material in which the said material passes over a heated aluminum cylinder having a hard, adherent, abrasion-resistant coating consisting substantially of aluminum oxide. Other objects of the invention will be apparent from the following specification and claims, and from the accompanying drawing.

I have discovered that aluminum or aluminum base alloy drying rolls which are provided with a coating of the type generally referred to in the art as an "oxide coating", have properties which make them highly suitable for use in the manufacture of cellulose films or sheets. The term "oxide coating" is used herein to designate an artificially produced coating consisting substantially of aluminum oxide on aluminum or aluminum base alloys, which coating is formed by a chemical or electrochemical treatment, and is of substantial thickness, as distinguished from the thin film of aluminum oxide which is naturally formed on aluminum surfaces by contact with the air. Such oxide coatings may be produced on aluminum surfaces by a number of well known methods, such as by immersing the article to be coated for a short time in a hot solution of an alkali carbonate containing a small amount of an inhibitor, such as a chromate, or by making the article the anode in an electrolytic cell in which the electrolyte consists of an acid solution, such as sulfuric acid, chromic acid, oxalic acid, or mixtures of these acids.

The characteristics of the coating vary somewhat with the methods used to produce them, particularly as to hardness. For my purposes, I prefer to use the methods which produce the harder, more adherent types of coating, and have found especially suitable the method in which the aluminum article to be coated is made the anode in an electrolyte containing about 5 to 35 per cent of sulfuric acid. However, other methods can also be used satisfactorily, and it is to be understood that I do not intend my invention to be limited to an oxide coating produced by any particular method.

Oxide coatings of the character produced by such methods are ordinarily hard, adherent, abrasion-resistant, and somewhat absorptive or adsorptive. Drying rolls equipped with such coatings have a surface to which sheets of cellulose

material will adhere slightly during their passage over the rolls without the necessity of using varnish or similar substances on the roll surfaces. The properties of the coating may be modified to some extent, if desired, by treatment in hot water for a short time to render the coating less pervious and absorptive or adsorptive. The water should preferably be at boiling temperature, although satisfactory results can be obtained in water at temperatures as low as 80° C. The time of treatment in hot water may also vary in duration. Periods of from 5 to 30 minutes may be satisfactory, depending upon the initial characteristics of the coating and on the extent to which it is desired to alter those characteristics.

It may be desirable that the frictional resistance of some of the drying rolls vary from that of other rolls in the same drying machinery. This result can be accomplished readily in accordance with my invention by controlling such variable factors as the type of treatment used to produce the oxide coating and the duration of the treatment in boiling water, if such treatment is used. Generally, rolls which have been subjected to a boiling water treatment offer less frictional resistance to the cellulose material than oxide coated rolls which have not been so treated. The degree of frictional resistance offered by the rolls can also be increased by subjecting them to a suitable roughening procedure prior to applying the oxide coating, as by etching or sand blasting, so long as the roll surface is not roughened to such an extent that the cellulose films are marred during their passage over the rolls.

The invention will be found described with reference to the accompanying drawing, in which a drying roll prepared in accordance with my invention is illustrated, part of the roll being cut away to show the coating.

In the drawing, the drying roll is shown as comprising a hollow aluminum cylinder 1 having on its external surface a coating 2 consisting substantially of aluminum oxide. It will be appreciated that the thickness of the coating is exaggerated for the purposes of illustration. In actual practice, a coating of from .0005 to .001 of an inch in thickness is ordinarily sufficient. However, any desired thickness of coating can be used. Although, in the drawing, the oxide coating is shown only on the external surface of the cylinder, it will be appreciated that other portions of the roll, such as the interior, may also be coated to advantage.

Drying rolls embodying my invention have a hard, abrasion-resistant coating which, though it may be scored by the sharp knives used to cut away tangled cellulose material from the machinery, will not burr or develop rough edges. They offer proper frictional resistance to the cellulose material passing over them, insuring efficient drying and stretching of the material, and the material may be readily stripped from them

when necessary. Furthermore, since the rolls are made of aluminum, a more uniform distribution of heat is obtained throughout.

As a specific example of my invention, an aluminum base alloy drying roll cylinder was provided with an oxide coating by making it the anode in an electrolytic cell in which a 15 per cent solution of sulfuric acid constituted the electrolyte. A current having a density of 15 amperes per square foot of cylinder surface to be coated was applied for 70 minutes, with the electrolyte maintained at a temperature of 70° C. The cylinder was then removed from the electrolyte, rinsed with water, and dried.

In another example of the invention, an aluminum base alloy drying roll cylinder was provided with an oxide coating, as described in the previous paragraph, and was then immersed in boiling water for 5 minutes, after which it was removed from the water and dried.

As used hereinabove and in the appended claims, the term "aluminum" includes aluminum and aluminum base alloys.

I claim:

1. A drying roll for drying non-fibrous cellulose material, said roll comprising an aluminum cylinder having on at least part of its surface a hard, adherent, abrasion-resistant coating consisting substantially of aluminum oxide.

2. A drying roll for drying non-fibrous cellulose material, said roll comprising an aluminum cylinder having on at least part of its surface a hard, adherent, abrasion-resistant coating consisting substantially of aluminum oxide, said coating having the characteristics of such a coating which has been immersed in water at a temperature of 80° to 100° centigrade for at least 5 minutes.

3. In the production of non-fibrous cellulose sheet, the step comprising passing such cellulose sheet over a heated aluminum surface, said surface having a hard, adherent, abrasion-resistant coating consisting substantially of aluminum oxide.

4. In the production of non-fibrous cellulose sheet, the step comprising drying such cellulose sheet by passing it over a heated aluminum surface, said surface having a hard, adherent, abrasion-resistant coating consisting substantially of aluminum oxide.

5. In the production of non-fibrous cellulosic pellicles, the step which comprises passing the same over a heated anodized aluminum surface.

6. In the production of non-fibrous cellulosic pellicles, the step which comprises drying said pellicles by passing the same over a heated, sealed, anodized aluminum surface.

7. In the production of non-fibrous cellulosic pellicles, the step which comprises drying said pellicles by passing the same over a heated, sealed, anodized aluminum surface.

RICHARD R. LAING.